

March 6, 1945.

R. LEPSOE

2,371,105

ATOMIZATION PROCESS

Filed Sept. 21, 1943



Inventor

Robert Lepsoe

64  
A. Harold Peches  
1774.

## UNITED STATES PATENT OFFICE

2,371,105

## ATOMIZATION PROCESS

Robert Lepsoe, Trail, British Columbia, Canada,  
assignor to The Consolidated Mining and  
Smelting Company of Canada, Limited,  
Montreal, Quebec, Canada, a corporation of  
Canada

Application September 21, 1943, Serial No. 503,231  
In Canada September 22, 1942

11 Claims. (Cl. 83—91)

This invention relates to a method and apparatus for the production of finely divided metal powder and is particularly directed to the production of the metal powders of magnesium and magnesium alloys.

Processes for the production of metal in powder form by subjecting a stream of the molten metal to the disintegrating action of a stream of gas under relatively high pressure impinged thereon are relatively well known and have been and are being used for the production of the metal powders of a number of metals.

In general, the methods of the prior art employ a bath of molten metal maintained at or above normal atmospheric pressure. The surface of the bath of molten metal may be covered with a flux to protect it from the action of the atmosphere to which it would otherwise be exposed. A relatively thin stream of molten metal is withdrawn from the molten bath and is disintegrated by the action of a stream of gas under relatively high pressure. The high velocity of the atomizing gas disintegrates the stream of molten metal into small globules which are simultaneously converted into solid form and carried as finely divided particles, by the force of the blast, into a collection chamber.

It is known that the metal powders of magnesium and magnesium alloys can be produced by subjecting a relatively thin stream of the molten metal to the disintegrating action of a jet of atomizing gas impinged, under relatively high pressure, on the stream of metal. However, in the actual production of the metal powders of magnesium and magnesium alloys on a commercial scale, there are a number of difficulties which are not present in the production of the powders of metals such as aluminum, zinc, copper and nickel, and which must be overcome if the production of the powdered magnesium or magnesium alloy free from impurities is to proceed safely on a commercially economic scale. For example, the dangers of fire and explosion are always present in the treatment of molten magnesium and every precaution must be taken to avoid them. A further difficulty resides in the tendency of the magnesium to react with most of the known gases to form compounds which are highly undesirable in the final product. For instance, pure nitrogen will react with molten magnesium at elevated temperatures to form magnesium nitride, and when the nitrogen contains small quantities of oxygen, as such or as water vapour, as is usual in commercial supplies of nitrogen, it is found that oxygen reacts with the

magnesium, causing it to burn and form magnesium oxide. This reaction raises the temperature locally and thereby increases the dangers of fire and explosion, due to oxidation and nitriding.

In the course of the reaction between the magnesium and the nitrogen, there is danger of fire and explosion in addition to the contamination of the product with highly undesirable impurities.

A still further difficulty, in the production of the metal powders of magnesium and magnesium alloys, resides in the presence, in the final product, of particles of the flux used to protect the surface of the molten bath from the action of the gases, particularly air, to which it is exposed.

10 15 The principal object of the present invention is to provide a method, and apparatus for carrying out the method, by which the metal powders of magnesium and magnesium alloys can be produced without danger of fire or explosion.

20 A further object of the invention is to provide a method and apparatus for the production of the metal powders of magnesium and magnesium alloys of a substantially uniform particle size and of a high degree of purity.

25 One of the principal features of the invention resides in the manner in which a relatively thin stream of molten metal, uncontaminated with flux, is withdrawn from a bath of molten magnesium or magnesium alloy, through a passageway

30 in a porous sleeve or nozzle impregnated with a flux whereby the exposed surface of the stream of metal, in passing through the nozzle, is in contact with the flux impregnating the nozzle and becomes coated with an extremely thin film of flux, and the stream of molten metal is, in effect, sheathed or enclosed in an extremely thin film of flux, whereafter a jet of gas under relatively high pressure is impinged on the stream of metal thereby disintegrating the molten metal into finely

35 40 divided particles which are carried, by the force of the blast, into a collection chamber. The thin film of flux in which the stream of metal is enclosed serves to protect the stream of molten metal from reaction with the gas in the powder chamber, and the danger of fire and the formation of compounds undesirable in the final product are avoided.

45 50 A further and preferred feature of the invention resides in the use of a flux which is of higher specific gravity than that of the bath of molten metal. The flux is in the form of a molten layer in the lower part of the vessel below the bath of molten metal, and surrounds the lower portion of the porous nozzle in the pot, whereby the flux is absorbed into the pores of the nozzle. As the

molten metal passes through the nozzle, it becomes coated with a thin film of flux with the result that the stream of metal issuing from the nozzle is effectively sheathed in a thin, uniform flux film. As the upper part of the nozzle extends above the layer of flux into the bath of molten metal, the metal stream issuing from the nozzle contains no lumps or particles of flux but, due to the method of operation, the stream of metal is provided with a protective film of flux. The pores of the nozzle remain constantly impregnated with flux during the operation of the method.

A still further feature of the invention resides in the design of apparatus suitable for carrying out the method and producing thereby metal powders of magnesium and magnesium alloys of substantially uniformly sized particles of high purity.

The manner in which I attain the above and other objects of this invention may be understood from the following description and accompanying drawing in which is illustrated a cross-sectional side elevation of a preferred form of apparatus suitable for carrying out the method.

Like reference characters refer to like parts throughout the specification and drawing.

The numeral 1 indicates a furnace setting preferably formed of insulating material such as fire brick. A metal pot or vessel 2 is received within the furnace setting, being carried on the walls of the setting by outwardly extending lugs 3. The vessel 2 may be heated in any one of several ways such as by oil or coal firing or by electricity. I prefer to provide electrical heating elements 4 between the outer walls of the vessel 2 and the furnace setting. The elements 4 are connected to a source of electrical energy through the leads 5 and 6.

The bottom of the pot 2 is drilled to form an opening approximately at the centre thereof into which is welded a downwardly extending sleeve 7 which is preferably tapered. A porous, refractory nozzle 8, preferably graphite, is fitted snugly into the sleeve 7. The nozzle 8 extends upwardly a short distance into the body of the pot and extends downwardly approximately flush with or slightly below the bottom of the sleeve 7. I prefer to taper the sleeve 7 slightly inwardly and the nozzle 8 is tapered correspondingly so that the nozzle fits snugly and tightly into the sleeve.

The nozzle 8 is drilled, preferably centrally, throughout its length to form a relatively narrow channel 9 which forms a passageway for the stream of molten metal. The furnace 1, the pot 2, and the heating elements 4, are preferably so designed that they form a portable unit.

The powder chamber 11 is of standard design, being provided with an opening at one end through which the jet 14 extends horizontally and a hopper-like collection chamber 12 at the end remote from the jet 14 wherein the metal powder is accumulated. A door 13 is provided in the base of the collection chamber 12 through which the metal powder may be removed. An opening 15 is provided in the uppermost wall of the collection chamber through which the gases may be withdrawn therefrom. A further opening is formed in the upper wall of the powder chamber above the inwardly extending end of jet 14. The opening is of sufficient size to receive, in snug fitting relationship, the tapered lower end of nozzle 8.

The portable furnace unit, comprising the pot 2, is placed at the end of the powder chamber

above the jet 14 in such a manner that the nozzle 8 fits snugly into the opening above the jet 14, in which position the atomizing gas, ejected under relatively high pressure from the jet 14, impinges, at substantially right angles, on the stream of metal, indicated by the numeral 10, issuing from the nozzle 8.

The installation and operation of the unit are relatively simple. The unit is placed in position on the upper wall of the powder chamber above the jet 14 and with the sleeve 7 in line with the opening directly above the atomizing jet. The pot 2 is then heated to a temperature above the melting temperature of the magnesium or magnesium alloy. While the pot is heating, the porous nozzle 8 may be fitted into position in sleeve 7, in which position the lower end of the nozzle may extend through the aforesaid opening a short distance into the powder chamber.

When the pot has been heated to its predetermined temperature, the flux is introduced into the pot, forming a layer of molten flux, indicated by the numeral 11, in the bottom thereof. The depth of the layer of flux is such that its upper surface is below the upper end of nozzle 8. A stopper attached to a rod (not shown) is inserted in the passageway in the nozzle and the pot is filled with magnesium or a magnesium alloy, indicated by the numeral 18. Powdered flux may be sprinkled over the surface of the molten bath to form a thin film of flux over the surface and thereby prevent exposure of the surface of the molten metal to the atmosphere. Before the molten metal is allowed to flow through the nozzle, the powder collecting system is thoroughly flushed with atomizing gas to remove all air. This may be done while the pot is being heated. The stopper may then be removed and, at the same time, the pressure of the atomizing gas, flowing through jet 14, may be raised to the desired operating pressure. The atomizing gas, under relatively high pressure, impinges on the stream of molten metal leaving the nozzle 8, thereby disintegrating the stream of metal into small globules which substantially instantaneously solidify into finely divided particles which are carried, by the force of the blast, into collection chamber 12.

The metal powder collected in chamber 12 may be removed periodically through clean-out door 13 provided for that purpose. The gas in the chamber 11-12 passes out through opening 15 and is passed through suitable dust collecting apparatus (not shown) to separate the entrained metal powder particles, after which it may be re-compressed and returned to the process.

The molten metal in pot 2 may be maintained at a substantially constant level by the continuous or intermittent addition of metal thereto.

Referring to the details of the process, the porous nozzle 8 may be formed of any one of a number of refractory materials capable of self-impregnation with the flux in which it is partially immersed. Very satisfactory results have been obtained from the use of graphite which is wettable by the flux but which is not reactive therewith or with the metal with which it is in contact.

The flux preferably has a higher specific gravity than that of the molten metal. It has been found that fluxes of lower specific gravity, such as lithium chloride, may evaporate, leaving the surface of the metal exposed to the atmosphere, with resultant oxidation. Another disadvantage of a lighter flux is that it will oxidize, forming a

product heavier than the metal, which settles through the bath of metal thereby contaminating the molten stream withdrawn through the nozzle and deleteriously affecting the fluidity of the bath.

Satisfactory results in the operation of the method may be obtained from any one of a number of fluxes, the composition of which may vary over a relatively wide range. In general, the flux is preferably composed of magnesium chloride, in combination with other chlorides or fluorides other than those which will so affect the surface tension of the flux that its protective properties are diminished. It has been found that most satisfactory results are obtained from the use of a flux composed of from 50% to 60% magnesium chloride and from 50% to 40% sodium chloride. A flux of this composition is of sufficiently high specific gravity that it remains as a layer in the bottom of the vessel in contact with the lower portion of the nozzle in the pot, and yet forms an extremely thin film over the surface of the bath of metal which protects the surface from the oxidizing action of the atmosphere. In the operation of the method, it has been found that there is a consumption of about one pound of flux for each ton of molten metal atomized.

The gas impinged on the stream of molten metal leaving the nozzle 8 and used to disintegrate the molten metal into finely divided particles is preferably nitrogen, carbon dioxide or mixtures thereof, containing as little free oxygen as possible, although it has been found that air can be used for short periods. An appreciable saving is effected by recirculating the exit gas from the collection chamber.

In the operation of the method, the upper end of the nozzle 8 extends into the bath of metal above the layer of flux, and the stream of metal, therefore, is not contaminated with particles of entrained flux or other foreign matter. The lower portion of the nozzle in the pot is immersed in the flux and, consequently, the pores of the nozzle are constantly maintained impregnated with the flux. As the stream of molten metal flows through the channel 9, the surface of the stream in contact with the walls of the channel acquires an extremely thin film of flux so that, in effect, the stream of molten metal is enclosed in the thin film of flux.

The thin film of flux which encloses the stream of molten metal issuing from the nozzle 8 makes it possible to overcome the difficulties hitherto associated with the production of the metal powders of magnesium and magnesium alloys. Ordinarily, magnesium will react readily with nitrogen or carbon dioxide at temperatures above the melting point of magnesium to form magnesium nitride or magnesium oxide with the attendant danger of fire and contamination of the final product with undesirable compounds. The thin film of flux enclosing the stream of metal prevents contact between the atomizing gas and the molten metal with the result that the dangers of fire and explosion are avoided and no undesirable compounds are formed which would contaminate the final product. It has been found in continuous operation of the method that magnesium metal heated to temperatures as high as 100 centigrade degrees above its melting point can be atomized with nitrogen, carbon dioxide, or mixtures thereof, without danger of fire and without the formation of compounds undesirable in the final product.

By operating at elevated temperatures, the molten metal is highly fluid and under the action of the atomizing gas, under relatively high pressure, disintegrates into finely divided particles of substantially uniform size.

The film of flux also serves as a lubricant causing the metal to flow smoothly through the nozzle 8 at temperatures lower than would be possible without the flux, thereby permitting operation of the method at lower temperatures, if desired. A lower temperature lessens the rate of oxidation of metal in the pot and also assists in maintaining a low temperature in the collection chamber.

15 The metal powders of magnesium-aluminum alloys can be produced successfully by the method and apparatus described hereinabove. As the percentage of aluminum in the alloy is increased, the specific gravity of the molten metal approaches that of the preferred magnesium chloride-sodium chloride flux until, in a magnesium-aluminum alloy containing about 50% aluminum, the flux would be lighter than the molten metal and would float on the surface of the metal in the pot. There is, of course, less danger of fire when treating magnesium alloys of high aluminum content but it has been found that by impregnating the nozzle with flux prior to commencing operations, adequate protection is provided until the supply of flux is depleted, thereby eliminating the danger of fire and obtaining the improved product described hereinabove.

30 It will be understood that the application of the present method and apparatus is not limited to the preferred embodiment described and illustrated herein. Various modifications of the invention may become apparent to those skilled in the art in the light of the teachings herein without departing from the scope of the invention as defined by the appended claims.

35 What I claim as new and desire to protect by Letters Patent of the United States is:

40 1. The method of producing metallic powders of magnesium and magnesium alloys which comprises passing a stream of molten metal through a porous nozzle impregnated with a flux comprising magnesium chloride, and thereafter disintegrating the stream of metal by the action of a jet of atomizing gas under relatively high pressure impinged thereon.

45 2. The method of producing the metal powders of magnesium and magnesium alloys which comprises enclosing a stream of the molten metal in a thin film of flux comprising magnesium chloride and thereafter disintegrating the stream of metal by the action of a jet of atomizing gas under relatively high pressure impinged thereon.

50 3. The method of producing the metal powders of magnesium and magnesium alloys which comprises maintaining, in separate layers in a vessel, a bath of molten metal and a molten flux comprising magnesium chloride, withdrawing a stream of molten metal from a portion of the bath remote from the flux and passing the stream of metal through a porous nozzle in contact with said flux, whereby the pores of said nozzle are impregnated with said flux and the surface of the stream of metal passing through said nozzle becomes coated with a thin film of said flux, and thereafter disintegrating the stream of metal by the action of a jet of an atomizing gas under relatively high pressure impinged thereon.

55 4. The method of producing the metal powders of magnesium and magnesium alloys which com-

prises maintaining, in separate layers in a vessel, a bath of molten metal and a magnesium chloride-sodium chloride flux, withdrawing a stream of molten metal from a portion of the bath remote from the flux and passing the stream of metal through a porous nozzle in contact with said flux, whereby the pores of said nozzle are impregnated with said flux and the surface of the stream of metal passing through said nozzle becomes coated with a thin film of said flux, and thereafter disintegrating the stream of metal by the action of a jet of an atomizing gas under relatively high pressure impinged thereon.

5. The method of producing the metal powders of magnesium and magnesium alloys which comprises maintaining, in separate layers in a vessel, a bath of molten metal and a molten flux comprising magnesium chloride and being of greater specific gravity than said metal, withdrawing a stream of molten metal from a portion of the bath remote from the flux and passing the stream of metal through a porous nozzle in contact with said flux, whereby the pores of said nozzle are impregnated with said flux and the surface of the stream of metal passing through said nozzle becomes coated with a thin film of said flux, and thereafter disintegrating the stream of metal by the action of a jet of an atomizing gas, under relatively high pressure, impinged thereon.

6. The method of producing the metal powders of magnesium and magnesium alloys which comprises maintaining, in separate layers in a vessel, a bath of molten metal and a magnesium chloride-sodium chloride flux, withdrawing a stream of molten metal from a portion of the bath remote from the flux and passing the stream of metal through a porous nozzle in contact with said flux whereby the pores of said nozzle are impregnated with said flux and the surface of the stream of metal passing through said nozzle becomes coated with a thin film of said flux, and thereafter disintegrating the stream of molten metal by the action of an atomizing gas, selected from the group consisting of nitrogen, carbon dioxide, and mixtures thereof, under relatively high pressure, impinged thereon.

7. In a process for the production of metallic powders of magnesium and magnesium alloys, the method of passing a stream of molten metal through a porous graphite nozzle impregnated with a flux comprising magnesium chloride whereby the surface of the stream of molten metal becomes coated with a thin film of flux, and thereafter disintegrating the stream of molten metal by the action of an atomizing gas, under relatively high pressure, impinged thereon.

8. Apparatus for the production of metallic powders which comprises a pot, and means for heating said pot, an opening in the base of said pot, a porous, graphite nozzle fitted into said opening and extending upwardly into said pot, a passageway extending through said nozzle, a layer of molten flux in the lower part of said pot, and a layer of molten metal above said flux, said nozzle extending through said flux into the bath of metal, whereby the pores of said nozzle are impregnated with said flux and the stream of metal is withdrawn from a portion of the bath remote from said flux, and means for disintegrating the stream of metal issuing from the passageway in said nozzle.

9. Apparatus for the production of metallic powders which comprises a pot, and means for heating said pot, an opening in said pot and a porous refractory nozzle fitted into said opening and extending into said pot, a passageway extending through said nozzle, a bath of molten metal and a layer of molten flux in said pot, said nozzle extending through said flux into the bath of metal whereby the pores of said nozzle are impregnated by said flux and the stream of metal is withdrawn from a portion of the bath remote from said flux, and means for disintegrating the stream of metal issuing from the passageway in said nozzle.

10. Apparatus for the production of metal powders which comprises a pot, and means for heating said pot, an opening in the base of said pot, a layer of molten flux in the lower part of said pot, and a layer of molten metal above said flux, a porous nozzle wettable by said flux fitted into said opening and extending upwardly through said flux into the bath of metal, whereby the pores of said nozzle are impregnated with said flux and the stream of metal is withdrawn from a portion of the bath remote from said flux, and means for disintegrating the stream of metal issuing from the passageway in the nozzle.

11. The method of reducing explosion and fire hazards in the production of metal powders of magnesium and magnesium alloys which comprises passing a stream of molten metal through a porous refractory nozzle impregnated with a flux comprising magnesium chloride whereby the surface of the stream of molten metal becomes coated with a thin film of flux, and thereafter disintegrating the stream of molten metal by the action of an atomizing gas, under relatively high pressure, impinged thereon.

ROBERT LEPSOE.